

## UNITED STATES PATENT OFFICE

1,941,039

## MAGNESIUM ALLOY

Alexander Luschenowsky, Berlin, Germany

No Drawing. Application December 14, 1931,  
Serial No. 581,050, and in Germany December  
17, 1930

1 Claim. (Cl. 75—1)

Magnesium alloys with zinc or zinc and manganese are already in use for several technical purposes. However, their application is limited on account of their tensile strength, especially with castings, being not very satisfactory. These known magnesium alloys also have no great resistance against chemical and corrosive attacks.

Besides they are inflammable, which renders their casting difficult and forms a great source of danger. Finally these alloys do not flow and especially can not be used for castings, which have thin walls.

The invention obviates these drawbacks by the addition of iron and silver or beryllium to alloys of the aforesaid type; it therefore refers to magnesium alloys with at least 80% Mg and Zn or Zn and Mn and Fe, Ag or beryllium.

The Mg, Zn, Fe, Ag alloys may contain up to 15% Zn, 2% Fe and 2% Ag, the rest being Mg.

20 The Mg, Zn, Mn, Fe, Ag alloys may contain up to 15% Zn, up to 3% Mn, up to 1% Fe and up to 1.5% Ag.

The simultaneous presence of Fe and Ag or Be produces a very satisfactory crystal-formation 25 and the structure of these alloys shows a fine, homogeneous and uniform grain.

The addition of Ag prevents an incomplete 30 equilibrium of the mixed crystals or with other words it prevents the "so-called" inter-crystalline liquation.

The uniform structure protects the alloys against corrosive attacks of the surface; the resistance against corrosion is improved by the fact, that the alloys with comparatively small 35 additions of other components already attain better qualities than the known Mg-alloys containing much higher percentages of foreign elements. Besides having a greater inertness against corrosion and chemical attacks, these al-

loys have far better mechanical capacities especially higher tensile strength, ductility, elongation and hardness. They are less inflammable, they flow well and can be easily cast; they can be mechanically worked with no difficulty, have 60 a very low spec. weight of about 1.7 and a silvery, wonderful colour.

The silver can be replaced, wholly or partly, by beryllium; this addition increases particularly 65 the hardness of these alloys.

The selection of the components used and their quantities depends mainly on the special application of the alloy, the maximum of spec. weight, which is allowable in the special case, 70 and the varying working conditions.

In order to manufacture the present alloys the following manner was found to give best results.

A preliminary alloy which contains the necessary amount of Zn, Fe, Ag or Zn, Fe, Be or Zn, 75 Fe, Ag, Be is added to the molten Mg or Mg—Mn alloy. In case manganese is used, it has been found advisable to divide the quantity of this metal and to add one part to the same to the magnesium and the other part to the preliminary 80 alloy of Zn, Fe, Ag or Zn, Fe, Be or Zn, Fe, Ag, Be; in such way a better distribution of the manganese is obtained.

Aluminium may be present up to 5%, silicon 85 only as an impurity.

What I claim is:

Magnesium-alloy containing not more than 15% and not less than 0.5% Zn, not more than 3% and not less than 0.01% Mn, not more than 1.5% and not less than 0.01% Fe, not less than 90 0.005% and not more than 1.5% Ag, the balance being Mg.

ALEXANDER LUSCHENOWSKY.